

## UNITED STATES PATENT OFFICE

2,337,013

## METHOD OF MAKING COATED PAPER

Donald B. Bradner, Mount Healthy, and William J. Montgomery, Hamilton, Ohio, assignors to The Champion Paper and Fibre Company, Hamilton, Ohio, a corporation of Ohio

No Drawing. Application July 6, 1940,  
Serial No. 344,234

4 Claims. (Cl. 117—103)

This invention relates to coated paper and methods of making same, and more particularly to coated paper having a "cast" surface such as described in Patent No. 1,719,166, issued July 2, 1929 to Donald B. Bradner, one of the present applicants.

The paper of the present invention is eminently adapted to the production of can and bottle labels, of cigarette and other packages, for fancy candy box wrappings, for carton liners, for book jackets, magazine covers, advertising folders and other uses.

As pointed out in the above mentioned patent, coated papers of especially high gloss and unusual smoothness may be obtained by the casting processes therein described.

The cast coated papers as described in the Bradner patent have frequently suffered from microscopic defects which detracted from the appearance and interfered with fine printing. Among the defects noticeable upon microscopic or naked eye examination of the paper may be mentioned the following:

*Trenches.*—This is a condition readily observed under a low power microscope, in which a coating, instead of being smooth and uniform, presents a surface containing shallow trenches that follow certain of the surface fibers of the underlying paper. When viewed with transmitted light these trenches are seen to be more transparent than the surrounding coating.

*Crevices.*—Microscopic irregular shaped holes in the coating having the appearance of shrinkage cracks.

*Holes.*—Microscopic rounded holes having the appearance of being caused by minute gas bubbles in the coating.

*Stipple.*—A condition of the coating readily seen by the naked eye by transmitted light. The coating is in thick and thin areas spaced a millimeter or two apart. This condition is often observable by reflected light.

*Cockle.*—A condition of the cast coated paper which has the cockled appearance of air dried bond paper as contrasted with a flat calendered paper.

We have discovered that all of these defects, notwithstanding their different and distinctive nature, are materially reduced, in fact practically eliminated by so controlling the flow or diffusion of the aqueous vehicle from the coating compositions into the paper stock, and the removal of the water through the back of the web, that no considerable proportion of the fibers in the paper is wetted at any time. Otherwise stated, in the

practice of our improved process we prevent deleterious swelling of the paper by limiting the rate of penetration of the water from the coating into the paper and by rapidly evaporating the water through the back of the sheet.

By a selection of paper stock and coating composition we can retard a rapid penetration of water from the coating into the sheet and by maintaining a high rate of evaporation through the back of the paper we rapidly remove whatever water that does diffuse into the paper. In this way deleterious swelling of the paper is prevented and defects in the surface of the cast coating are eliminated or reduced to an extent to permit the manufacture of a product suitable for high grade printing.

The paper stock should be of a kind which is not too rapidly wet by the coating composition employed, and it should retard rapid absorption of the coating vehicle into the paper. For this purpose, a dense, well formed, hard-sized paper is desirable. By hard-sized paper we mean paper containing an agent which resists rapid absorption of water, as for example a paper containing a considerable amount of rosin sizing which has been precipitated with alum. As an example of what we mean by hard-sized paper we may mention the equivalent of a paper of a basic weight of 45 pounds per ream of 500 sheets 25 x 38 inches and having a sizing value in excess of 15 seconds as measured by the Valley size test. Paper stocks which are well formed and relatively dense are preferred for the present purpose over widely formed, bulky, porous stocks, as they show a greater resistance to the penetration of water from the coating.

With regard to the selection of coating compositions, those of high total solids are in general desirable for our purposes. We prefer to use coating compositions considerably higher in solids content than are customarily used in making mineral coated paper. For example, we prefer to use coating compositions having a solids content in excess of 45% and advantageously of the order of 50% to 55%. By the use of coating compositions of high solids content, less water is available for penetration into the paper and the higher viscosities usually accompanying high solids coatings also retard rapid flow of the water into the sheet. The ingredients used in the coating compositions may be those commonly employed in the usual paper coating compositions.

The water which diffuses into the paper must be rapidly evaporated through the back of the web in order to prevent accumulation of water in

the paper, which would cause substantial swelling of the fibers. This may be accomplished by providing a blast of hot air on the back of the web. Under these conditions it appears that the amount of water in the body of the stock is maintained at such a low value that the fibers are not wetted sufficiently to produce a swelling which is harmful to the coating. It is possible that the mechanism of the process is that, although the surface layer of the paper next to the coating may become thoroughly wet, substantially all of the water may vaporize through the sheet from this very thin layer, so that there is little or no diffusion of liquid water into the body of the paper.

In general it is advisable to apply the coating to the paper web only a very short time before contact with the finishing surface in order to reduce the degree of penetration of water into the paper.

It will be evident that a combination of all three of the above mentioned factors will ordinarily give the most beneficial results. For example, a combination of a water-resistant body stock, high solids coating, and rapid evaporation is particularly desirable. Considerable variation, however, in any of these factors or conditions is permissible provided compensation is made in the other factors and conditions. For example, reducing the water impenetrability of the paper stock may be offset by increasing the solids or by increasing the viscosity of the coating composition, or both. Also, by increasing the rate of evaporation a higher rate of absorption may be permitted.

Although this invention has been described primarily in connection with the application of a coating composition directly to the paper and the subsequent drying of the coating while in contact with a solid finishing surface, the process of the invention may also be carried out in accordance with the method described in our prior Patent No. 2,029,273. In carrying out this embodiment of the present invention, the coating composition is applied directly to the finishing surface and the web of substantially dry paper is contacted with the still wet coating on the finishing surface and the coating is transferred to the paper during the time the coating is setting. Deleterious swelling of the fibers in the paper is prevented in the same manner as has been described in connection with the method of directly applying the coating to the paper, namely, by a proper selection of the paper stock and coating composition and by increasing the rate of evaporation.

The expression "cast surface" is used in the appended claims to designate coating surfaces, whatever their composition, which have been set from a plastic condition in contact with a solid non-adhering casting surface in the manner described in the patent to Brander, No. 1,719,166 and the patent to Bradner and Montgomery, No. 2,029,273 so that they have substantially the same finish as the casting surface itself.

We claim:

1. A method of making cast surfaced coated paper which comprises applying to one face of a paper web a layer, in excess of two pounds dry

weight per thousand square feet of surface, of coating composition comprising pigment and adhesive in aqueous suspension, contacting the coated surface of said web with a casting surface, 5 bringing a current of air in contact with the exposed surface of the paper web to evaporate the water therefrom, and maintaining the rate of evaporation relatively high with respect to the rate of absorption of water by the paper web, whereby the water content of the paper web is insufficient to cause a significant swelling of the fibres.

2. A process of manufacturing cast surfaced coated paper having a coating in excess of two pounds dry weight per thousand square feet of surface, which comprises applying to one face of a paper web having a low rate of water absorption a layer of coating composition comprising mineral pigment in aqueous suspension, pressing 15 the face of the paper web against a casting surface and drying the coating while in contact with the casting surface until the coating no longer adheres to such surface, said drying being accomplished by bringing a current of air of relatively low water content against the exposed surface of the web at a rate such as to maintain the water content of the paper during the drying operation below an amount which will cause a significant swelling of the fibres of the paper 20 web.

3. A process of manufacturing cast surfaced coated paper having a coating in excess of two pounds dry weight per thousand square feet of surface which comprises applying to one face of a paper web a layer of coating composition comprising mineral pigment and adhesive in aqueous suspension having a solids content in excess of 45%, pressing the face of the paper web against a casting surface and drying the coating 25 while in contact with the casting surface until the coating no longer adheres to such surface, said drying being accomplished by bringing a current of air of relatively low water content against the exposed surface of the web at a rate such as to maintain the water content of the paper during the drying operation below an amount which will cause a significant swelling of the fibres of the paper web.

4. A process of manufacturing cast surfaced coated paper having a coating in excess of two pounds dry weight per thousand square feet of surface which comprises applying to one face of a paper web having a low rate of water absorption a layer of coating composition comprising mineral pigment and adhesive in aqueous suspension and having a solids content in excess of 45%, pressing the face of the paper web against a casting surface and drying the coating while in contact with the casting surface until the coating no longer adheres to such surface, said drying being accomplished by bringing a current of air of relatively low water content against the exposed surface of the web at a rate such as to maintain the water content of the paper during the drying operation below an amount which will cause a significant swelling of the fibres of the paper web.

DONALD B. BRADNER.

WILLIAM J. MONTGOMERY.